

Feb. 9, 1943.

J. BARAB

2,310,344

BLASTING CARTRIDGE

Filed April 18, 1941



FIG. - 1



FIG. - 2

JACOB BARAB  
INVENTOR.

BY *Cleveland B. Mackay*

## UNITED STATES PATENT OFFICE

2,310,344

## BLASTING CARTRIDGE

Jacob Barab, Wilmington, Del., assignor to  
 Hercules Powder Company, Wilmington, Del.,  
 a corporation of Delaware

Application April 18, 1941, Serial No. 389,124

8 Claims. (Cl. 102—24)

This invention relates to an improved blasting cartridge and to methods of production thereof. It relates more particularly to a blasting cartridge surrounded by a compressible admixture which provides a cushioning action for the initial explosive shock.

It is the principal object of this invention to provide a blasting cartridge enclosed in a sheath comprising a compressible cushioning admixture. A further object of this invention is to provide a sheath comprised of an admixture which is compressible and which contains a flame-quenching salt. A further object of this invention is to provide a comparatively low density admixture which may be packed into a tubular sheath for use around an explosive cartridge.

A further object of this invention is to provide an explosive cartridge surrounded by a comparatively low density, tubular sheath which will cushion the initial shock of the explosion. A still further object of this invention is to provide an explosive cartridge which is surrounded by a tubular sheath of compressible material that will give improved blasting results in operations such as coal mining.

Other and further objects will be apparent hereinafter.

The cushioning of the initial shock of a blasting explosion with a compressible, cushioning material in accordance with this invention is of particular importance for explosive cartridges subject to use in producing high percentages of lump material such as is desired in coal mining. After the initial shock of the explosive has been absorbed by the cushioning material, the expanding gases released by the explosion further expand, but without a shattering force, into the cleavage planes of the seam being blasted with a resulting pushing action which breaks up the structure in such a manner that large firm lumps are obtained. Without the cushioning material about the explosive, the shattering force causes a large amount of pulverized material to be produced. In particular, for example, lump coal brings higher prices and any improvement which will give a larger percentage of lump in any given blast constitutes a highly desirable improvement in the blasting operation necessary in coal mining.

The improvement in blasting cartridges described in accordance with this invention may be accomplished with any desired form of explosives, but will be found most advantageous in connection with, for example, the dynamites developed for use in coal mining. The shattering

effect of coal mining explosives, for example, the permissible dynamites, when fired in direct contact with coal, while not of the high order of that obtained with straight dynamites, is, nevertheless, undesirable. By sheathing these explosives, especially the permissibles, a higher percentage of lump coal is obtained.

The improved explosive cartridge which provides the advantage related above in the mining of lump coal may be produced in accordance with the present invention by surrounding an explosive cartridge with a sheath comprising an admixture of diatomite, such as diatomaceous earth, kieselguhr, tripolite, infusorial earth and the like, a binder and a flame-quenching salt. The binders which I have found desirable for use with the diatomite may be materials having adhesive properties or material which form a matrix such as, for example, dextrin, clay, sodium silicate, waste sulfite liquor, wood pulp, such as kraft pulp or sulfite pulp, asbestos fiber, balsa, bagasse, and other similar binding materials. The flame-quenching salt which I have found to be adaptable for use in my admixture may be, for example, sodium bicarbonate, sodium chloride, boric acid, ground gypsum, borax, calcium chloride or the like.

The admixture prepared in accordance with this invention may be formed into a tubular sheath by packing it into an annular ring within a substantially rigid tube so that the internal diameter thereof is equivalent to the diameter of the explosive cartridge which is to be inserted within the tubular member. The formed sheathing will be semi-rigid and have a cellular, favose structure. The packing of the material may be accomplished by machines such as, for example, described in the co-pending application of R. B. Smith and K. Wassen, Serial No. 273,301, filed May 12, 1939.

Having now indicated in a general way the nature and purpose of this invention, there follows a more detailed description of preferred embodiments thereof with reference to the accompanying drawing in which Fig. 1 represents a cushioning sheath partially in section and containing an explosive cartridge, and Fig. 2 is a view of the cushioning sheath of Fig. 1, on line 2—2.

Referring now to the drawing, the assembled article of this invention comprises a blasting cartridge 1 surrounded by a cushioning sheath 2 comprising a packed, homogeneous material 3 retained in position by a surrounding tube 4. The explosive cartridge 1 comprises an explosive

composition 5 wrapped in paper 6 which is crimped 7 at the end.

If desirable, a cap 8 may be placed over either or both ends of the assembly. The cap will be found desirable when a unitary exposure charge is manufactured. The cap may be placed on the end of the cushioning sheath as shown in Fig. 1 and either be composed of a sheet of material such as cardboard or the like or composed of the compressible admixture 3 which surrounds the explosive cartridge. If it is desirable, the cap may be formed in the shape of a plug and inserted in the end of the sheath 2 proper. In such instances the sheath 2 will be slightly longer than the explosive cartridge which is to be used. The plug may be retained by any adhesive, taping or similar expedient.

The thickness of the cushioning material may be varied to provide varying amounts of cushioning effect. A thickness of about  $\frac{1}{8}$  to about  $\frac{3}{4}$  inch is desirable for most purposes. Thus, a sheath to fit around a  $1\frac{1}{4}$  by 8 inch dynamite cartridge will be about  $1\frac{1}{3}$  inches, inside diameter, and about  $1\frac{1}{2}$  inches to about  $1\frac{3}{4}$  inches outside diameter. This sheath may, of course, be about the same length as the cartridge and open on both ends in order to aid propagation of the explosive, or the ends of the cartridge may be closed with caps or plugs described hereinbefore, and made either of cardboard or of the sheathing composition. The closing of the ends of the cartridge slightly retards the propagation of detonation from one cartridge to another, but, when only one cartridge is to be used in the explosion, the closed end sheath is desirable.

The diatomite which is found preferable for use in the sheath of this invention is known by many names in the industry and is produced in many sections of the country.

In the specification and claims, the term diatomite is here used in its generally accepted sense, i. e., diatomite is the name now generally given to a mineral substance composed of the tiny skeletal remains of diatoms which are microscopic, flowerless, water plants related to the algae. This residuum diatomite is essentially hydrous amorphous silica.

Common names for diatomite are: Diatomaceous earth, tripolite, kieselguhr, and infusorial earth. Strictly speaking, however, the latter material is not truly a diatomite, as it is composed of the fossil remains of infusoria, which usually do not occur with the diatomaceae. Other synonyms for diatomite are: Diatomaceous silica, kieselmehl, bergmehl, diatomene-peelite, polirschiefer, moler, molera, molererde, desmid earth, fossil flour, mountain flour, farine fossil, white peat, radiolarian earth, chalk rock, ceyssatite, randanite, and tellurine; also various diatomite products of individual companies are known by their own trade names.

The sheathing in accordance with this invention may comprise as high as about 50% diatomite, but will preferably contain between about 30 and about 40% diatomite with the remaining percentage comprising a flame quenching salt and minor amounts of binder. The sheaths found most desirable for commercial use are composed of an admixture of 35% diatomite, 65% sodium bicarbonate with just sufficient dextrin binder to form a packable composition which upon drying will not crumble.

In order to illustrate the various preferable embodiments of the invention, the following examples are given.

### Example I

Sheaths were made from the following admixture: 600 pts. sodium bicarbonate, 400 pts. diatomite, 400 pts. sodium silicate solution—5 1 part in 12 parts of water by packing into a spiral-wound paper tube. The total amount of water present will be coordinated to give most desirable packing properties. The wall thickness of the packed sheaths was 0.233" and the average weight of a  $1\frac{1}{4}$ " x 8" sheath, exclusive of the paper tube, was approximately 115 g. Similar sheaths composed of only sodium bicarbonate and a dextrin binder weighed 154 g. The apparent densities of the two types of sheaths were 0.79 g./cc. and 1.05 g./cc. respectively.

### Example II

Sheaths were made from the following composition: 700 pts. sodium bicarbonate, 300 pts. diatomite, 250 pts. dextrin binder.

This composition produced a sheath for a  $1\frac{1}{4}$ " x 8" explosive cartridge which had a dry weight of 125 g. with a wall thickness of approximately 0.23" and a density of 86 g./cc. The dextrin binder used was prepared by making an aqueous solution containing about 6-8% dextrin and 2-3% borax. If desired and in order to facilitate packing, the binding solution may be further diluted, or in some instances, it may be used in a more concentrated form. The borax was added as a preservative but is not essential.

### Example III

Sheaths were made from a composition comprising 650 parts of sodium bicarbonate and 350 parts of diatomite in which the amount of binder was varied over a wide range. The cartridge had a dry weight of 120 g. and a density of 82 g./cc. 40 The amount of binder was not essential, however, small amounts of binder produced sheaths which had a tendency to crumble while excessive binder made the admixture difficult to pack.

45 The two sheaths described in Examples I and II, after being dried, were crushed in a hydraulic press to determine their strength. The method was to place the sheaths between two saddles 1 inch wide and apply hydraulic pressure until 50  $\frac{1}{8}$  inch movement took place. On this test the crushing strength of the sheaths was about 60 to 70 pounds which is sufficient strength to withstand handling, packing, and shipping.

55 The advantages of the sheaths of this invention are that they are very easily manufactured, since the admixtures pack easily and dry quickly. Further, the ingredients are economically and easily obtainable in all sections of the country and do not require expensive processing. Further, it has been found that the strength of the sheaths produced is high enough so that sheathing may be prepared at an explosive plant and shipped without insertion of a support within the tube. The sheathings may be shipped in 60 normal cases, and, upon arriving at the destination, are not broken or crushed. The possibility of shipping sheaths without supports within the tube allows a reduction of freight rates and does away with the necessity of removing the supports whenever the tubes are to be used. Of course, it is possible to ship the sheath around explosive cartridges, but in doing this, the freight rates are much higher since explosive materials carry premium freight rates. Likewise, it is oftentimes desirable to use explosive

cartridges without the sheath around the cartridge, especially when overburden of slate must be broken out of the way to contact the coal face. By shipping the sheath and explosive cartridges in separate containers, it is possible to use one type explosive within a mine, and this is advantageous since the fewer materials there are to be isolated, the more efficient the operation of the mine becomes.

It will be appreciated that the above details and examples are given merely for the purpose of illustrating my invention and are not intended to limit the invention. Moreover, many variations in the compositions and procedures employed may be made without departing from the scope of the invention.

The present application is a continuation-in-part of my applications, Serial Nos. 225,342, now U. S. Patent No. 2,227,059, and 345,712, filed August 17, 1938, and July 16, 1940, respectively.

What I claim and desire to protect by Letters Patent is:

1. An improved blasting assembly including an explosive cartridge surrounded by a pre-formed, annular, tubular sheath comprising between about 30% and about 50% diatomite, and a flame-quenching salt, said sheath characterized by a semi-rigid, cellular, favose structure which is adapted to provide a cushioning action for the initial explosive shock.

2. An improved blasting assembly including an explosive cartridge surrounded by a pre-formed, annular, tubular sheath comprising between about 30% and about 50% diatomite, a binder, and a flame-quenching salt, said sheath characterized by a semi-rigid, cellular, favose structure which is adapted to provide a cushioning action for the initial explosive shock.

3. An improved blasting assembly including an explosive cartridge surrounded by a pre-formed, annular, tubular sheath comprising between about 30% and about 50% diatomite, a matrix, and a flame-quenching salt, said sheath characterized by a semi-rigid, cellular, favose

structure which is adapted to provide a cushioning action for the initial explosive shock.

4. An improved blasting assembly including an explosive cartridge surrounded by a pre-formed, annular, tubular sheath comprising between about 20% and about 50% and a flame-quenching salt, said sheath characterized by a semi-rigid, cellular, favose structure which is adapted to provide a cushioning action for the initial explosive shock.

5. An improved blasting assembly including an explosive cartridge surrounded by a pre-formed, annular, tubular sheath comprising between about 30% and about 50% diatomite and sodium bicarbonate, said sheath characterized by a semi-rigid, cellular, favose structure which is adapted to provide a cushioning action for the initial explosive shock.

6. An improved blasting assembly including an explosive cartridge surrounded by a pre-formed, annular, tubular sheath comprising between about 30% and about 50% diatomite, dextrin, and a flame-quenching salt, said sheath characterized by a semi-rigid, cellular, favose structure which is adapted to provide a cushioning action for the initial explosive shock.

7. An improved blasting assembly including an explosive cartridge surrounded by a pre-formed, annular, tubular sheath comprising between about 30% and about 50% diatomite and wood pulp, and a flame quenching salt, said sheath characterized by a semi-rigid, cellular, favose structure which is adapted to provide a cushioning action for the initial explosive shock.

8. An improved blasting assembly including an explosive cartridge surrounded by a pre-formed, annular, tubular sheath comprising between about 30% and about 50% diatomite, sodium bicarbonate, and dextrin, said sheath characterized by a semi-rigid, cellular, favose structure which is adapted to provide a cushioning action for the initial explosive shock.

JACOB BARAB.